

Jan. 21, 1930.

E. B. LE MARE

1,744,478

COOLING AND ANNEALING OF GLASS IN STRIP FORM AND APPARATUS THEREFOR

Filed Nov. 12, 1924

Fig. 1.



Fig. 2.



Inventor:

E. B. Le Mare

By  
Rogers, Kennedy, Campbell

Atty's.

Fig. 3.



## UNITED STATES PATENT OFFICE

ERNEST BRISTOW LE MARE, OF ST. HELENS, ENGLAND, ASSIGNOR TO PILKINGTON BROTHERS LIMITED, OF LIVERPOOL, ENGLAND, A BRITISH COMPANY

## COOLING AND ANNEALING OF GLASS IN STRIP FORM AND APPARATUS THEREFOR

Application filed November 12, 1924, Serial No. 749,421, and in Great Britain November 19, 1923.

This invention relates to the cooling and annealing of glass in strip form and apparatus therefor and has for its object to prevent the warping of the strip and to maintain it flat during cooling and solidification.

If a sheet of glass, during its transition from the plastic to the solid condition, be cooled more rapidly from one surface than from the other, the sheet on complete solidification, will warp.

In order, therefore, that the strip be maintained flat, it is essential that the cooling be symmetrical with reference to the centre plane of the strip; that is to say, that the last layer of the strip to solidify be the central layer.

It is not, however, essential that the rates of cooling from the two surfaces be equal at all stages of the transition, provided that any inequality at one stage be compensated by an opposite inequality at another stage.

The above mentioned period of transition starts at the point of formation of the strip and continues to a point in the lehr, and the length of strip between these two points may be divided into two portions, that between the point of formation and the lehr, and that in the lehr itself.

In the following specification and the claims, the term "lehr" is used to denote a kiln in which the glass is annealed and is supported on a bed, such as a series of rollers, adapted to cause the glass to travel from the hot to the colder end. Further, since glass has no definite point of solidification, it is assumed to be solidified when it has reached a condition in which it can acquire a permanent strain.

According to this invention, the cooling of the upper and lower surfaces of the strip of glass in the lehr, while in its transition period, is controlled, one relatively to the other, in such a manner that, before the solidification point of the whole strip is reached, the strip has been symmetrically cooled, whatever may have been the relative amounts of cooling from the two surfaces of the strip at its entrance to the lehr.

In the accompanying drawings:—

Figure 1 is a vertical longitudinal section,

partly broken away, of a portion of a lehr constructed in accordance with, and adapted for carrying out, the invention, the said section being taken on the line 1—1 of Figure 2 looking towards the left of that figure;

55

Figure 2 is a transverse section of the same on the line 2—2 of Figure 1 looking towards the right of that figure, and drawn to a scale twice that to which Figure 1 is drawn, and

60

Figure 3 is an alternative form of the right-hand portion of Figure 1.

The strip of glass 1 rests on the bed of rollers 2 in the lehr 3, the left-hand end of Figure 1 representing the hot end of the lehr. Above the strip of glass 1, are three muffles 4, 4 and 5 and below it are five muffles 6, 6, 7, 7, and 8. These muffles are supplied with hot gases from a number of flues, the two top outer muffles 4,4 being supplied from the flues 9, 9, the top muffle 5 from the flues 10, 10 and the bottom muffles from the flues 11.

65

The top muffles 4, 5 are heated by gas jets from a gas flue 12 and the bottom muffles 6, 7 and 8 are heated by gas jets from the gas flues 13. Each flue is provided with air controlling dampers 14 and gas controlling dampers 18.

70

At that point in the lehr at which the strip has become solidified throughout, the top muffles 4, 5 are connected to exhaust flues 15, 16 respectively, a damper 17 being provided to control the amount of hot gases passing through each muffle.

75

The bottom muffles 6, 7 and 8 continue to the far end of the lehr and are there connected to an exhaust flue in the ordinary way, these muffles providing for the heating of the lehr after the solidification point of the glass.

80

The relative rates of cooling of the upper and lower surfaces of the strip can be controlled in the above described construction, 90 by varying the pull in the exhaust ports 15, 16 and by varying the amount of heating gases introduced into all or any of the flues 9, 10 and 11.

95

The control of the said relative rates of cooling and the heating of the lehr after the solidification point of the glass, may be secured in many alternative ways. Thus, the heating of the lehr after the solidification point may be quite independent of that up 100

to the said point, as shown in Figure 3, where 19 and 20 are heating ports leading to muffles 21 which are provided with exhaust ports towards the end of the lehr. Alternatively, 5 in the arrangement shown in Figure 1, the heating in the latter portion of the lehr may be maintained substantially independent of that up to the solidification point, by maintaining constant the supply of heat to the 10 bottom muffles and also the total supply of heat through all the ports 9 and 10, the necessary relative control of the heating above and below the glass being secured by increasing the heat supplied through the ports 9 and 15 10 near the beginning of the lehr and correspondingly reducing that through the ports further down the lehr, or vice versa.

In the length of lehr up to the solidification point of the glass, any number of hot 20 gas supply ports may be provided for both the top and bottom muffles and, in cases where the difference in the rates of cooling of the 25 upper and lower surfaces of the strip is not great, the number of inlet ports may be reduced from that shown, and may differ in the upper and lower muffles. Thus, the strip may 30 reach the lehr in such condition that sufficient control is secured by a single inlet port in each upper muffle and by two in each lower muffle, or vice versa.

Since it may result from the treatment of the strip before it reaches the lehr, that the amounts of cooling of the upper and lower surfaces of the strip differ by amounts which 35 are different for the edge portions from what they are for the central portion of the strip, a plurality of muffles preferably are provided either above or below or both above and below the strip. In the particular construction 40 of lehr shown in the drawings, three muffles are shown above and five below, the heat supplied to the strip by each muffle being independently controllable as described above. By means of this independent control, the 45 relative rates of cooling of the upper and lower surfaces of the strip may be controlled so as to be different for portions of the strip nearer the edges from what it is for portions nearer the centre of the strip.

50 A similar though less complete difference in control may be secured by employing a plurality of muffles above and a single muffle below or vice versa.

The supply of heat to the lehr, though 55 preferably effected by means of muffles may be by direct admission of hot gases and the term "hot gases" is to be taken to include either gases in a state of combustion or the products of their combustion.

60 Having described my invention, I declare that what I claim and desire to secure by Letters Patent is:—

1. Process of cooling continuous glass strip in a lehr in which the products of gaseous 65 combustion are introduced into portions of

the lehr both above and below the glass strip near the entrance end of the lehr, the amount of heat thereby supplied to the upper surfaces of the edge portions of the strip relatively to that supplied to their lower surfaces being controlled and the amount of heat supplied to the upper surface of the central portion of the strip relatively to that supplied to its lower surface being independently controlled, the said controls being to secure "symmetrical cooling" before the strip "solidifies".

2. Process of cooling continuous glass strip in a lehr in which products of gaseous combustion are introduced into portions of the 80 lehr both above and below the glass strip near the entrance end of the lehr, the amount of heat thereby supplied to the upper surfaces of the edge portions of the strip relatively to that supplied to their lower surfaces being controlled and the amount of heat supplied to the upper surface of the central portion of the strip relatively to that supplied to its lower surface being independently controlled, the said controls being to secure "symmetrical cooling" before the strip "solidifies" and withdrawing the said products by flues which are independent for the upper and lower portions of the lehr.

3. A lehr for continuous glass strip comprising heating means in the first portion before the strip "solidifies", means adapted to control the relative amount of heat supplied to retard the cooling of the two surfaces of the strip in said portion, and heating means in the latter portion substantially independent of the heating means in the said first portion.

4. A lehr for continuous glass strip comprising a plurality of hot gas supply ports longitudinally of the lehr adapted to supply heat to one surface of the strip in the first portion of the lehr before the strip "solidifies", at least one port adapted to supply heat to the other surface of the strip before it "solidifies", means adapted to control the relative amount of heat supplied to the two surfaces, and heating means in the latter portion of the lehr substantially independent of the heating means in the said first portion.

5. A lehr for continuous glass strip comprising means adapted to supply a controllable amount of heat to the upper surface of the strip, means adapted to supply a controllable amount of heat to the lower surface of the strip and means adapted to control the amount of heat supplied to the central portion of the strip relatively to that supplied to the edge portions thereof.

6. A lehr for continuous glass strip comprising heating means in the first portion before the strip "solidifies", means adapted to control the relative amount of heat supplied to retard the cooling of the two surfaces of the strip in said portion, means adapted to

supply heat to the portions of the strip nearer to the edge and means substantially independent thereof adapted to supply heat to portions nearer to the centre of the strip, and heating means in the latter portion of the lehr substantially independent of the heating means in the said first portion.

7. A horizontal lehr for continuous glass strip, comprising muffles on each side of the strip, means independent with respect to the two sides of the strip for introducing hot gases into the muffles and means adapted to control the relative amount of heat so supplied to the muffles on the two sides of the strip.

8. A lehr for continuous glass strip comprising a plurality of muffles transversely of the lehr adapted to supply heat to one surface of the strip before it "solidifies", at least one muffle adapted to supply heat to the other surface of the strip, and means adapted to control the relative amount of heat so supplied to the two surfaces.

9. A lehr for continuous glass strip comprising muffles into which hot gases are introduced for supplying heat to the first portion of the lehr to retard the cooling of the two surfaces of the strip before it solidifies, means adapted to control the relative amount of heat so supplied to the two surfaces, and heating means in the latter portion of the lehr substantially independent of the heating means in the said first portion.

10. A lehr for continuous glass strip comprising muffles adapted to supply heat to retard the cooling of the two surfaces of the strip at different portions thereof respectively nearer to the edge and nearer to the centre, and means adapted to control the relative amount of heat supplied to said different portions.

In testimony whereof I have affixed my signature hereto.

ERNEST BRISTOW LE MARE.